# EUROPEAN PATENT SPECIFICATION

(11) **EP 1 705 266 B1**
(45) Date of publication and mention of the grant of the patent: **02.09.2009**
(21) Application number: 06251532.5
(22) Date of filing: 22.03.2006
(51) Int. Cl.: C23C 24/04, F01D 5/00

(54) **Applying bond coat to engine components using cold spray**
Auftragen einer Haftbeschichtung auf Motorbauteile mittels eines Kaltsprühverfahrens
Dépôt d'une couche de liaison sur des organes de machine par pulverisation à froid

(30) Priority: 23.03.2005 US 88380
(43) Date of publication of application: 27.09.2006
(73) Proprietor: United Technologies Corporation, Hartford Connecticut 06101 (US)
(72) Inventor: DeBiccari, Andrew, North Branford, CT 06471 (US); Freling, Melvin, West Hartford, CT 06117 (US); Haynes, Jeffrey D., Stuart, FL 33496 (US)
(74) Representative: Leckey, David Herbert

(56) References cited:
- EP-A- 1 398 394
- EP-A2- 1 659 195
- GB-A- 2 394 479
- US-A- 5 302 414
- US-A1- 2002 073 982
- US-A1- 2003 126 800
- US-A1- 2004 110 021
- US-B1- 6 365 222

## Description

### BACKGROUND OF THE INVENTION

### (1) Field of the Invention

The present invention relates to a process for applying a coating to a combustion chamber liner, used in an engine.

### (2) Prior Art

Currently, bond coats are applied using low-pressure plasma spray (LPPS). Operation and maintenance of LPPS systems is expensive and time consuming, limiting throughput. Also, LPPS requires a vacuum chamber. The size of a given chamber limits the size of the parts that can be processed.

Cold gas dynamic spraying or "cold spray" has been recently introduced as a new metallization spray technique to deposit powder metal without inclusions onto a substrate. A supersonic jet of helium and/or nitrogen is formed by a converging/diverging nozzle and is used to accelerate the powder particles toward the substrate to produce cold spray deposits or coatings. Deposits adhere to the substrate and previously deposited layers through plastic deformation and bonding. U.S. Patent Nos. 5,302,414 and 6,502,767 illustrate cold gas dynamic spraying techniques.

A method of lining an aluminium cylinder block by cold spraying is described in US 2002/0073982. A method of cold spraying a mandrel is disclosed in EP-A-1659195 which forms prior art under Art 54(3) EPC.

### SUMMARY OF THE INVENTION

Accordingly, it is an object of the present invention to provide a process for applying a coating to a component used in an engine which reduces cycle times and maintenance costs.

It is a further object of the present invention to provide a process as above which can be used with any size component.

The foregoing objects may be attained using the process of the present invention.

In accordance with the present invention, there is provided a process as claimed in claim 1.

Other details of the technique for applying a bond coat to engine components using cold spray of the present invention are set forth in the following detailed description and the accompanying drawings wherein like reference numerals depict like elements.

### BRIEF DESCRIPTION OF THE DRAWINGS

FIG. 1 is a schematic representation of an apparatus for depositing cold sprayed powder metal materials onto a component used in an engine.

### DETAILED DESCRIPTION OF THE PREFERRED EMBODIMENT(S)

The present invention relates to a process for applying a coating to a combustion chamber liner used in rocket engines.

The cold spray process for depositing powdered materials onto portions of a component which needs to be restored is advantageous in that it provides sufficient energy to accelerate particles to high enough velocities such that, upon impact, the particles plastically deform and bond to the surface of the component being restored or onto a previously deposited layer. The cold spray process allows the build up of a relative dense coating or structural deposit. Cold spray does not metallurgically transform the particles from their solid state.

When preparing to coat an article or component, it is often necessary to remove any pre-existing coating on the article or component. Any suitable stripping technique may be used to remove any pre-existing coating and to provide a fresh surface to which a coating material can be deposited. For example, any pre-existing coating may be stripped using mechanical or chemical techniques.

Referring now to FIG. 1, there is shown a system 8 for depositing a powder coating material onto a surface 24 of an article or component 10 to be coated.

The system 8 includes a spray gun 22 having a converging/diverging nozzle 20 through which the powdered coating material is sprayed onto the surface 24. The article 16 is a combustion chamber liner, and is formed from a nickel or copper-based alloy. During the coating operation, the article or component 10 may be held stationary or may be articulated, rotated, or translated by any suitable means (not shown) known in the art.

In the process of the present invention, the material to be deposited is a powdered material. The powdered coating material is a copper alloy such as a copper-chromium alloy or a copper-chromium-aluminum alloy. The coating material may form a stand alone coating or a bond coat for metallic and ceramic overcoats.

The powdered coating materials that are used to form the deposit on the surface 24 may have a diameter of 5-80 microns, preferably a diameter of 10 microns or less if the alloy material being deposited is hard. In a most preferred embodiment, the powdered coating materials has a diameter in the range of from about 5.0 microns to 10 microns. Smaller particle sizes enable the achievement of higher particle velocities. Below 5 microns in diameter, the particles risk getting swept away from the surface 24 due to a bow shock layer above the surface 24, i.e. insufficient mass to propel the particle through the bow shock. The narrower the particle size distribution, the more uniform the particle velocity will be. This is because the smaller particles in the spray/plume will hit the slower, larger ones and effectively reduce the velocity of both.

The particles to be deposited may be accelerated to supersonic velocities using compressed gas, such as a gas selected from the group consisting of helium, nitrogen, another inert gas, and mixtures thereof. Helium is a preferred gas because it produces the highest velocity due to its low molecular weight.

The bonding mechanism employed by the process of the present invention for transforming the powdered coating material into a deposit is strictly solid state, meaning that the particles plastically deform but do not melt. Any oxide layer that may have formed on the particles, or is present on the surface 24, or is present in a previously deposited layer, is broken up and fresh oxide-free contact is made at very high pressures.

The powdered coating material used to form the deposit may be fed to the spray gun 22 using any thermal spray feeder known in the art with the capability to feed the powder or the stated size. One such feeder that may be used is manufactured by Powder Feed Dynamics of Cleveland, Ohio. This feeder has an auger type feed mechanism. Fluidized bed feeders and barrel roll feeders with an angular slit may also be used.

In the process of the present invention, the feeder may be pressurized with a gas selected from the group consisting of helium, nitrogen, another inert gas, and mixtures thereof. Feeder pressures are generally 15 psi (103 kPa) above the main gas or head pressures, which pressures are usually in the range of from 200 psi (1.38 MPa) to 500 psi (3.45 MPa), depending on the powdered coating material composition. The main gas is preferably heated so that gas temperatures are in the range of from 600 degrees Fahrenheit (315°C)to 1200 degrees Fahrenheit (649°C). If desired, the main gas may be heated as high as approximately 1250 degrees Fahrenheit (677°C) depending on the material being deposited. The gas may be heated to keep it from rapidly cooling and freezing once it expands past the throat of nozzle 20. The net effect is a surface temperature on the article or component 10 of about 115 degrees Fahrenheit (46°C) during deposition. Any suitable means known in the art may be used to heat the gas.

To deposit the powdered coating material, the nozzle 20 may pass over the surface 24 of the article or component 10. The number of passes is a function of the thickness of the material to be applied. The process of the present invention is capable of forming a deposit having any desired thickness.

The main gas that is used to deposit the powdered metal particles onto the surface 24 may be passed through the nozzle 20 via inlet 30 at a flow rate of from 0.001 SCFM (0.028 1/Min) to 50 SCFM (1416 l/Min), preferably in the range of from 15 SCFM (425 1/Min) to 35 SCFM (991 l/Min). The foregoing flow rates are preferred if helium is used as the main gas. If nitrogen is used by itself or in combination with helium as the main gas, the nitrogen may be passed through the nozzle 20 at a flow rate of from 0.001 SCFM (0.028 l/Min) to 30 SCFM (849 l/Min), preferably from 4.0 SCFM (113 l/Min) to 30 SCFM (849 l/Min), more preferably 4.0 SCFM (113 l/Min) to 8.0 SCFM (227 l/Min).

The main gas temperature may be in the range of from 600 degrees Fahrenheit (315°C) to 1200 degrees Fahrenheit (649°C), preferably from 700 degrees Fahrenheit (371°C) to 1000 degrees Fahrenheit (539°C), and most preferably from 725 degrees Fahrenheit (385°C) to 900 degrees Fahrenheit (482°C).

The pressure of the spray gun 22 may be in the range of from 200 psi (1.38 MPa) to 500 psi (3.45 MPa), preferably from 200 psi (1.38 MPa) to 400 psi (2.76 MPa), and most preferably from 275 psi (1.80 MPa) to 375 psi (2.59 MPa). The powdered coating material is preferably fed from a hopper, which is under a pressure in the range of from 10 (69 kPa) to 50 psi (345 kPa) higher than the specific main gas pressure, preferably 15 psi (103 kPa) higher, to the spray gun 22 via line 34 at a rate in the range of from 10 grams/min to 100 grams/min, preferably from 10 grams/min to 50 grams/min.

The powdered coating material is fed to the spray gun 22 using a non-oxidizing carrier gas. The carrier gas may be introduced via inlet 30 at a flow rate of from 0.001 SCFM (0.028 1/Min) to 50 SCFM (1416 l/Min), preferably from 8.0 SCFM (227 1/Min) to 15 SCFM (425 l/Min). The foregoing flow rate is useful if helium is used as the carrier gas. If nitrogen by itself or mixed with helium is used as the carrier gas, a flow rate of from 0.001 SCFM (0.028 1/Min) to 30 SCFM (849 1/Min), preferably from 4.0 to 10 SCFM (113 l/Min to 238 l/Min), may be used.

The spray nozzle 20 is held at a distance from the surface 24. This distance is known as the spray distance and may be in the range of from 10 mm. to 50 mm.

The velocity of the powdered coating particles leaving the spray nozzle 20 may be in the range of from 825 m/s to 1400 m/s, preferably from 850 m/s to 1200 m/s.

The process of the present invention is advantageous over the current LPPS processes. For example, in LPPS, the powder is melted. In the process of the present invention, the powder is not melted. Still further, LPPS requires the use of a vacuum chamber which limits the size of the article or component which can be coated. The process of the present invention does not require a vacuum chamber and may be performed in the open. As a result, there is no restriction on the size of the article or component which can be coated. In LPPS, it is possible to have deposits which include oxides that may render the coating brittle. In the process of the present invention, no such oxides are formed. Still another advantage of the cold spray process of the present invention is that the as-deposited coating is at least 97% dense. Still further, coated articles may be capable of having a bond strength capable of 10 ksi (68.95 N/mm²).

When the cold spray process is used to apply a bond coat, an additional coating layer or layers may be formed over the bond coat. Any suitable technique known in the art may be used to apply the overcoat layer(s). The overcoat materials make be metallic or ceramic in composition.

The cold spray process offers many other advantages over other processes. Since the powders are not heated to high temperatures, no oxidation, decomposition, or other degradation of the feedstock materials occurs. Other potential advantages include the formation of compressive residual surface stresses and retaining the microstructure of the feedstock. Also, because relatively low temperatures are used, thermal distortion of the substrate will be minimized. Because the feedstock is not melted, cold spray offers the ability to deposit materials that cannot be sprayed conventionally due to the formation of brittle intermetallics or a propensity to crack upon cooling or during subsequent heat treatments.

## Claims

1. A process for applying a coating to a component (10) comprising the steps of:
providing a component (10) having at least one surface (24) to be coated, said component being a combustion chamber liner formed from a nickel-based alloy or a copper-based alloy; and
depositing at least one layer of powder coating copper based alloy material onto said at least one surface using a non-oxidizing carrier gas so that said powder coating material plastically deforms without melting and bonds to said at least one surface upon impact with said at least one surface.

2. The process according to claim 1, wherein said depositing step comprises providing said powder coating material in particle form having a particle size no greater than 10 microns and wherein said depositing step comprises accelerating said particles to a speed in the range of from 825 m/s to 1400 m/s.

3. The process according to claim 1, wherein said depositing step comprises providing said powder coating material in particle form having a particle size in the range of from 5.0 microns to 10 microns and wherein said accelerating step comprises accelerating said particles to a speed in the range of from 850 m/s to 1200 m/s.

4. The process according to claim 1 or 2, wherein said depositing step further comprises feeding said powdered coating material to a spray nozzle at a feed rate of from 10 grams/min to 100 grams/min using a carrier gas selected from the group consisting of helium, nitrogen, another inert gas, and mixtures thereof.

5. The process according to claim 4, wherein said feeding step comprises feeding said metal powder to said spray nozzle at a feed rate of from 10 grams/min to 50 grams/min.

6. The process according to claim 4 or 5, wherein said carrier gas is helium and said feeding step comprises feeding helium to said nozzle at a flow rate of from 0.028 l/min (0.001 SCFM) to 1416 l/min (50 SCFM).

7. The process according to claim 6, wherein said feeding step comprises feeding said helium to said nozzle at a flow rate in the range of from 227 l/min (8.0 SCFM) to 425 l/min (15 SCFM).

8. The process according to claim 4 or 5, wherein said carrier gas comprises nitrogen and said feeding step comprises feeding said nitrogen to said nozzle at a flow rate of from 0.028 1/min (0.001 SCFM) to 849 l/min (30 SCFM).

9. The process according to claim 8, wherein said feeding step comprises feeding said nitrogen to said nozzle at a flow rate of from 113 l/min (4.0 SCFM) to 283 l/min (10 SCFM).

10. The process according to any of claims 4 to 9, wherein said depositing step comprises passing said powdered coating particles through said nozzle using a main gas selected from the group consisting of helium, nitrogen, another inert gas, and mixtures thereof at a main gas temperature in the range of from 315°C (600 degrees Fahrenheit) to 649°C (1200 degrees Fahrenheit) and at a spray pressure in the range of from 1.38 MPa (200 psi) to 3.45 MPa (500 psi).

11. The process according to claim 10, wherein said passing step comprising passing said powdered coating particles through said nozzle at a main gas temperature in the range of from 371°C (700 degrees Fahrenheit) to 538°C (1000 degrees Fahrenheit) at a spray pressure in the range of from 1.38 MPa (200 psi) to 276 Spa (400 psi).

12. The process according to claim 10, therein said main gas temperature is in the range of from 385°C (725 degrees Fahrenheit) to 482°C (900 degrees Fahrenheit) at a spray pressure in the range of from 1.90 MPa (275 psi) to 2.59 MPa (375 psi).

13. The process according to claim 10, 11 or 12, wherein said main gas comprises helium and said passing step comprises feeding said helium to said nozzle at a flow rate in the range of from 0.028 l/min (0.001 SCFM) to 1416 l/min (50 SCFM).

14. The process according to claim 13, wherein said helium feeding step comprises feeding said helium to said nozzle at a flow rate in the range of from 425 l/min (15 SCFM) to 991 l/min (35 SCFM).

15. The process according to claim 10, 11 or 12, wherein said main gas comprises nitrogen and said passing step comprises feeding said nitrogen to said nozzle at a feed rate in the range of from 0.028 l/min (0.001 SCFM) to 849 l/min (30 SCFM).

16. The process according to claim 15, wherein aid nitrogen feeding step comprises feeding said nitrogen to said nozzle at a feed rate in the range of from 113 l/min to 227 l/min (4.0 to 8.0 SCFM).

17. The process according to any preceding claim, wherein said depositing step comprises forming a bond coat on said component (10) having a bond strength in the range up to 68.95 N/MN² (10 ksi) or greater.

18. The process according to any preceding claim, wherein said depositing step comprises depositing a coating which is at least 97% dense on said component.

19. The process according to any preceding claim wherein said copper based alloy is a copper-chromium alloy.

20. The process according to any of claims 1 to 19 wherein said copper based alloy is a copper-chromium-aluminum alloy.

## Patentansprüche

1. Verfahren zum Auftragen einer Beschichtung auf ein Bauteil (10), folgende Schritte aufweisend:
Bereitstellen eines Bauteils (10) mit mindestens einer zu beschichtenden Oberfläche (24), wobei das Bauteil eine Verbrennungsraum-Auskleidung ist, die aus einer Legierung auf Nickelbasis oder einer Legierung auf Kupferbasis hergestellt ist; und
Abscheiden mindestens einer Schicht aus Pulverbeschichtungs-Legierungsmaterial auf Kupferbasis auf der mindestens einen Oberfläche unter Verwendung eines nichtoxidierenden Trägergases, so dass sich das Pulverbeschichtungsmaterial plastisch verformt ohne zu schmelzen und sich beim Auftreffen auf die mindestens eine Oberfläche mit der mindestens einen Oberfläche verbindet.

2. Verfahren nach Anspruch 1, bei dem der Schritt des Abscheidens ein Bereitstellen des Pulverbeschichtungsmaterials in Partikelform mit einer Partikelgröße von nicht größer als 10 µm aufweist, und bei dem der Schritt des Abscheidens ein Beschleunigen der Partikel auf eine Geschwindigkeit in dem Bereich von 825 m/s bis 1400 m/s aufweist.

3. Verfahren nach Anspruch 1, bei dem der Schritt des Abscheidens ein Bereitstellen des Pulverbeschichtungsmaterials in Partikelform mit einer Partikelgröße in dem Bereich von 5,0 µm bis 10 µm aufweist, und bei dem der Beschleunigingsschritt ein Beschleunigen der Partikel auf eine Geschwindigkeit in dem Bereich von 850 m/s bis 1200 m/s aufweist.

4. Verfahren nach Anspruch 1 oder 2, bei dem der Schritt des Abscheidens außerdem ein Zuführen des pulverförmigen Beschichtungsmaterials zu einer Spritzdüse mit einer Zuführgeschwindigkeit von 10 Gramm/min bis 100 Gramm/min unter Verwendung eines Trägergases, das ausgewählt wird aus der Gruppe, die aus Helium, Stickstoff, einem anderen Inertgas und Gemischen davon besteht, aufweist.

5. Verfahren nach Anspruch 4, bei dem der Schritt des Zuführens ein Zuführen des Metallpulvers zu der Spritzdüse mit einer Zuführgeschwindigkeit von 10 Gramm/min bis 50 Gramm/min aufweist.

6. Verfahren nach Anspruch 4 oder 5, bei dem das Trägergas Helium ist, und der Schritt des Zuführens ein Zuführen von Helium zu der Düse mit einer Strömungsgeschwindigkeit von 0,028 l/min (0,001 SCFM) bis 1416 l/min (50 SCFM) aufweist.

7. Verfahren nach Anspruch 6, bei dem der Schritt des Zuführens ein Zuführen des Heliums zu der Düse mit einer Strömungsgeschwindigkeit in dem Bereich von 227 l/min (8,0 SCFM) bis 425 l/min (15 SCFM) aufweist.

8. Verfahren nach Anspruch 4 oder 5, bei dem das Trägergas Stickstoff aufweist, und der Schritt des Zuführens ein Zuführen des Stickstoffs zu der Düse mit einer Strömungsgeschwindigkeit von 0,028 l/min (0,001 SCFM) bis 849 l/min (30 SCFM) aufweist.

9. Verfahren nach Anspruch 8, bei dem der Schritt des Zuführens ein Zuführen des Stickstoffs zu der Düse mit einer Strömungsgeschwindigkeit von 113 l/min (4,0 SCFM) bis 283 l/min (10 SCFM) aufweist.

10. Verfahren nach einem der Ansprüche 4 bis 9, bei dem der Schritt des Abscheidens ein Führen der pulverförmigen Beschichtungspartikel durch die Düse unter Verwendung eines Hauptgases, das ausgewählt wird aus der Gruppe, die aus Helium, Stickstoff, einem anderen Inertgas und Gemischen davon besteht, bei einer Hauptgastemperatur in dem Bereich von 315 °C (600 Grad Fahrenheit) bis 649 °C (1200 Grad Fahrenheit) und bei einem Spritzdruck in dem Bereich von 1,38 MPa (200 psi) bis 3,45 MPa (500 psi) aufweist.

11. Verfahren nach Anspruch 10, bei dem der Schritt des Führens ein Führen der pulverförmigen Beschichtungspartikel durch die Düse bei einer Hauptgastemperatur in dem Bereich von 371 °C (700 Grad Fahrenheit) bis 538 °C (1000 Grad Fahrenheit) bei einem Spritzdruck in dem Bereich von 1,38 MPa (200 psi) bis 276 MPa (400 psi) aufweist.

12. Verfahren nach Anspruch 10, bei dem die Hauptgastemperatur in dem Bereich von 385 °C (725 Grad Fahrenheit) bis 482 °C (900 Grad Fahrenheit) bei einem Spritzdruck in dem Bereich von 1,90 MPa (275 psi) bis 2,59 MPa (375 psi) liegt.

13. Verfahren nach Anspruch 10, 11 oder 12, bei dem das Hauptgas Helium aufweist, und der Schritt des Führens ein Zuführen des Heliums zu der Düse mit einer Strömungsgeschwindigkeit in dem Bereich von 0,028 l/min (0,001 SCFM) bis 1416 1/min (50 SCFM) aufweist.

14. Verfahren nach Anspruch 13, bei dem der Schritt des Zuführen von Helium ein Zuführten des Heliums zu der Düse mit einer Strömungsgeschwindigkeit in dem Bereich von 425 l/min (15 SCFM) bis 991 l/min (35 SCFM) aufweist.

15. Verfahren nach Anspruch 10, 11 oder 12, bei dem das Hauptgas Stickstoff aufweist, und der Schritt des Führens ein Zufuhren des Stickstoffs zu der Düse mit einer Zuführgeschwindigkeit in dem Bereich von 0,028 l/min (0,001 SCFM) bis 849 l/min (30 SCFM) aufweist.

16. Verfahren nach Anspruch 15, bei dem der Schritt des Zuführens von Stickstoff ein Zuführen des Stickstoffs zu der Düse mit einer Zufiihrgeschwindigkeit in dem Bereich von 113 l/min bis 227 l/min (4,0 bis 8,0 SCFM) aufweist.

17. Verfahren nach irgendeinem vorangehenden Anspruch, bei dem der Schritt des Abscheidens ein Ausbilden einer Bindungsbeschichtung auf dem Bauteil (10) mit einer Bindungsfestigkeit in dem Bereich von bis zu 68,95 N/MN² (10 ksi) oder größer aufweist.

18. Verfahren nach irgendeinem vorangehenden Anspruch, bei dem der Schritt des Abscheidens ein Abscheiden einer Beschichtung, die eine Dichte von mindestens 97 % hat, auf dem Bauteil aufweist.

19. Verfahren nach irgendeinem vorangehenden Anspruch, bei dem die Legierung auf Kupferbasis eine Kupfer-Chrom-Legierung ist.

20. Verfahren nach irgendeinem der Ansprüche 1 bis 19, bei dem die Legierung auf Kupferbasis eine Kupfer-Chrom-Aluminium-Legierung ist.

## Revendications

1. Procédé pour appliquer un revêtement à un composant (10) comprenant les étapes suivantes :
obtention d'un composant (10) ayant au moins une surface (24) à recouvrir, ledit composant étant une chemise de chambre de combustion formée d'un alliage à base de nickel ou d'un alliage à base de cuivre ; et
dépôt d'au moins une couche de matériau de revêtement en poudre en alliage à base de cuivre sur ladite au moins une surface en utilisant un gaz vecteur non oxydant de telle sorte que ledit matériau de revêtement en poudre se déforme plastiquement sans fondre et adhère à ladite au moins une surface lors d'un impact avec ladite au moins une surface.

2. Procédé selon la revendication 1, dans lequel ladite étape de dépôt comprend l'obtention dudit matériau de revêtement en poudre sous forme de particules ayant une taille de particules ne dépassant pas 10 µm, et dans lequel ladite étape de dépôt comprend l'accélération desdites particules jusqu'à une vitesse comprise dans la gamme de 825 m/s à 1400 m/s.

3. Procédé selon la revendication 1, dans lequel ladite étape de dépôt comprend l'obtention dudit matériau de revêtement en poudre sous forme de particules ayant une taille de particules comprise dans la gamme de 5,0 µm à 10 µm, et dans lequel ladite étape d'accélération comprend l'accélération desdites particules jusqu'à une vitesse comprise dans la gamme de 850 m/s à 1200 m/s.

4. Procédé selon la revendication 1 ou 2, dans lequel ladite étape de dépôt comprend en outre l'introduction dudit matériau de revêtement en poudre dans une buse de pulvérisation à une vitesse d'introduction de 10 grammes/min à 100 grammes/min en utilisant un gaz vecteur choisi dans le groupe constitué par l'hélium, l'azote, un autre gaz inerte et les mélanges de ceux-ci.

5. Procédé selon la revendication 4, dans lequel ladite étape d'introduction comprend l'introduction de ladite poudre métallique dans ladite buse de pulvérisation à une vitesse d'introduction de 10 grammes/min à 50 grammes/min .

6. Procédé selon la revendication 4 ou 5, dans lequel ledit gaz vecteur est l'hélium et ladite étape d'introduction comprend l'introduction d'hélium dans ladite buse à un débit de 0,028 l/min (0,001 SCFM) à 1416 l/min (50 SCFM).

7. Procédé selon la revendication 6, dans lequel ladite étape d'introduction comprend l'introduction dudit hélium dans ladite buse à un débit compris dans la gamme de 227 l/min (8,0 SCFM) à 425 l/min (15 SCFM).

8. Procédé selon la revendication 4 ou 5, dans lequel ledit gaz vecteur comprend de l'azote et ladite étape d'introduction comprend l'introduction dudit azote dans ladite buse à un débit de 0,028 l/min (0,001 SCFM) à 849 l/min (30 SCFM).

9. Procédé selon la revendication 8, dans lequel ladite étape d'introduction comprend l'introduction dudit azote dans ladite buse à un débit de 113 l/min (4,0 SCFM) à 283 l/min (10 SCFM).

10. Procédé selon l'une quelconque des revendications 4 à 9, dans lequel ladite étape de dépôt comprend le passage desdites particules de revêtement en poudre à travers ladite buse en utilisant un gaz principal choisi dans le groupe constitué par l'hélium, l'azote, un autre gaz inerte et les mélanges de ceux-ci à une température de gaz principal comprise dans la gamme de 315°C (600 degrés Fahrenheit) à 649°C (1200 degrés Fahrenheit) et à une pression de pulvérisation comprise dans la gamme de 1,38 MPa (200 psi) à 3,45 MPa (500 psi).

11. Procédé selon la revendication 10, dans lequel ladite étape de passage comprend le passage desdites particules de revêtement en poudre à travers ladite buse à une température de gaz principal comprise dans la gamme de 371°C (700 degrés Fahrenheit) à 538°C (1000 degrés Fahrenheit) à une pression de pulvérisation comprise dans la gamme de 1,38 MPa (200 psi) à 2,76 MPa (400 psi).

12. Procédé selon la revendication 10, dans lequel ladite pression de gaz principal se situe dans la gamme de 385°C (725 degrés Fahrenheit) à 482°C (900 degrés Fahrenheit) pour une pression de pulvérisation comprise dans la gamme de 1,90 MPa (275 psi) à 2,59 MPa (375 psi).

13. Procédé selon la revendication 10, 11 ou 12, dans lequel ledit gaz principal comprend de l'hélium et ladite étape de passage comprend l'introduction dudit hélium dans ladite buse à un débit compris dans la gamme de 0,028 l/min (0,001 SCFM) à 1416 l/min (50 SCFM).

14. Procédé selon la revendication 13, dans lequel ladite étape d'introduction d'hélium comprend l'introduction dudit hélium dans ladite buse à un débit compris dans la gamme de 425 l/min (15 SCFM) à 991 l/min (35 SCFM).

15. Procédé selon la revendication 10, 11 ou 12, dans lequel ledit gaz principal comprend de l'azote et ladite étape de passage comprend l'introduction dudit azote dans ladite buse à une vitesse d'introduction comprise dans la gamme de 0,028 l/min (0,001 SCFM) à 849 l/min (30 SCFM).

16. Procédé selon la revendication 15, dans lequel ladite étape d'introduction d'azote comprend l'introduction dudit azote dans ladite buse à une vitesse d'introduction comprise dans la gamme de 113 l/min à 227 l/min (4,0 à 8,0 SCFM).

17. Procédé selon l'une quelconque des revendications précédentes, dans lequel ladite étape de dépôt comprend la formation d'une couche d'accrochage sur ledit composant (10) ayant une force d'adhésion comprise dans une gamme allant jusqu'à 68,95 N/mm² (10 ksi) ou plus.

18. Procédé selon l'une quelconque des revendications précédentes, dans lequel ladite étape de dépôt comprend le dépôt d'un revêtement qui présente une densité d'au moins 97 % sur ledit composant.

19. Procédé selon l'une quelconque des revendications précédentes, dans lequel ledit alliage à base de cuivre est un alliage cuivre-chrome.

20. Procédé selon l'une quelconque des revendications 1 à 19, dans lequel ledit alliage à base de cuivre est un alliage cuivre-chrome-aluminium.
